

Nov. 27, 1934.

S. A. POLLOCK

1,982,122

METHOD OF NITRATING CELLULOSE

Filed April 12, 1932



Inventor:  
Samuel Alexander Pollock,  
By  
Byrnes, Stibbles, Parmelee & Blenko,  
Atty.

## UNITED STATES PATENT OFFICE

1,982,122

## METHOD OF NITRATING CELLULOSE

Samuel Alexander Pollock, London, England

Application April 12, 1932, Serial No. 604,854  
In Great Britain March 18, 1930

9 Claims. (Cl. 260—145)

The present invention consists of improvements in or relating to methods of nitrating cellulose and an object of the invention is to produce cheaply and conveniently a nitrated product in the form of separate relatively thin sheets having very uniform physical and chemical characteristics.

The invention is particularly applicable to the production of thin sheets of nitrated cellulose for use as separators in electric batteries and for making solutions of nitro-cellulose, for example, for producing acid-resisting varnishes.

According to the present invention a method of preparing separate relatively thin sheets of nitrated cellulose comprises placing in a nitrating bath relatively thin sheets of cellulose fibre paper interleaved with acid-proof spacing sheets provided with projections and recesses giving the nitrating fluid access to both sides of the sheets of cellulose.

Preferably the cellulose sheets are in the form of pure cotton fibre paper and are not more than 100th of an inch thick while the spacers are conveniently of aluminium, for example, corrugated sheet aluminium. Preferably the sheets lie in vertical or substantially vertical planes when immersed in the bath.

In one form of the invention the interleaved sheets and spacers are assembled in a box or cage capable of being lowered into and raised out of a nitrating bath and provided with apertures to allow the nitrating fluid to flow freely into the box among the sheets.

By means of the invention a nitrated cellulose paper is produced of which the composition is very uniform. It is found that ordinary methods of introducing paper into nitrating baths are liable to result in great variation of nitration and porosity which greatly affects the suitability of the product for use as battery separators and its complete solubility in ordinary nitro-cellulose solvents.

It is found that important factors in the process are the simultaneous access of nitrating acids to both sides of the paper, rapid and complete penetration of acid into all the fibres of the paper, rapid absorption by the concentrated acid of the water produced by the chemical reaction with the cellulose, control of the heat produced by the chemical reaction, and rapid removal of the acid from the nitrated paper at the end of the nitration. Spacers of aluminium besides being substantially acid-resisting assist substantially in the distribution of the heat produced by the reaction.

An apparatus suitable for carrying out my invention is illustrated in the accompanying drawing.

As shown in the drawing the box 10 which is of aluminium is of rectangular form with a perforated bottom 11, perforated end walls 12, and handles 15. Single sheets 13 of paper are interleaved with thin corrugated aluminium sheets 14 of approximately the same dimensions and placed in the box parallel with its side walls. The box is designed to hold a convenient number of sheets, for example 120, standing on edge on the bottom of the box.

The box containing the paper and aluminium sheets is placed for about an hour in a drying oven maintained at a temperature slightly above 100 degrees centigrade until the paper is thoroughly dried. The box with its contents is then removed from the oven and when cooled to a temperature of about 15 degrees centigrade is submerged for about 30 minutes in a bath containing a mixture of sulphuric and nitric acids and water of the following approximate composition:—

Sulphuric acid 44.3 per cent., nitric acid 37.4 per cent., water 18.2 per cent. If sulphuric acid of 1.84 specific gravity and nitric acid of 1.42 specific gravity are used the above composition is obtained by taking two parts of sulphuric acid to three parts of nitric acid. The chemical reaction which takes place between the acids and the cellulose is principally controlled by the concentration of the acid in the bath and the temperature of the bath. I find that when the bath

is maintained at a temperature of about 15 degrees centigrade and a sufficient volume of acid is used to completely submerge the aluminium box and its contents the paper acquires in the time mentioned a definite increase in weight of about 55 per cent., when weighed after complete washing in water and drying. It also acquires the valuable qualities of great strength in the wet condition and a high degree of toughness and flexibility which it retains indefinitely in battery acid of the usual strength, extremely low in electrical resistance when immersed in the battery electrolyte, and a favourable degree of porosity which completely prevents the finest sediment escaping from sheaths made from this material or causing a bridge or short-circuit between oppositely charged plates.

The satisfactory working and maintenance of the acid bath in order to effect economy of acids and obtain a uniform product which is of great importance requires detailed explanation. The compound of cellulose esters which is formed

60

65

70

75

80

85

90

95

100

105

110

with the acids reaches an equilibrium with the concentration of acid in the bath so that the quantities of cellulose and acids in the bath when equilibrium is reached effect the result obtained.

5 For example, 1000 grams of cellulose combine with about 778 grams of nitric acid under these conditions of concentration and temperature to form about 1565 grams of the particular cellulose ester and about 222 grams of water. The 10 consumption of acid and the formation of water as the result of the reaction necessitate a readjustment of the bath before it can be satisfactorily used again to produce a similar result. On the 15 assumption that 1000 grams of pure cellulose paper is treated at one time in the bath the required adjustment may be calculated as follows:—As a first step 778 grams of nitric acid should be restored to the bath to replace the amount used by the previous batch of paper. Using 20 nitric acid of 1.5 specific gravity containing 94 per cent pure acid the amount required is  $778 \times 100$  divided by 94=827 grams. The addition of this acid will unavoidably add 6 per cent. of 227 grams of water, i. e. about 49 grams of water 25 containing the acid. Therefore the bath becomes diluted by the addition of 222 grams of water from the reaction plus 49 grams introduced by the nitric acid addition. In order to restore the water content to its original value of 18.2 per cent. a 30 sufficient quantity of mixture of concentrated sulphuric and nitric acids in the original ratio of 44.3 to 37.4 must be added to balance the excess of 271 grams water. This ratio of acids will be obtained by taking sulphuric acid of 1.84 specific 35 gravity (95.6 per cent strength) and nitric acid of 1.500 specific gravity (94 per cent strength) in the following quantities:—

$$443 \times 100 \div 95.6 = 463.4$$

40 grams sulphuric acid of 1.84 S. G. and

$$374 \times 100 \div 94 = 398$$

grams nitric acid of 1.5 S. G. The corresponding amount of water to these quantities according 45 to the original ratio is 182 grams but these quantities only contain  $463.4 \times 4.4 \div 100$  plus

$$398 \times 6 \div 100 = 44.26$$

grams water. The balance of water therefore required by these quantities of acid to make up the origin ratio is 182 minus 44.26=137.74 grams, i. e. to balance such an increment of 137.74 grams of water brought into the bath by reaction the above amount of acids would 50 be required, and to balance the actual increment of 271 grams water the foregoing quantities would 55 need to be increased in the ratio of 271 to 137.74.

I have found in practice that some additional water is unavoidably introduced by incomplete 60 drying of the paper and by absorption of water from the air and also that some additional nitric acid leaves the bath in the form of vapour. To compensate for these variations I have found that the foregoing calculated amounts should be increased by 20 per cent and after a full day's operation the bath should be analyzed in known manner to determine the amounts of the acids remaining in the bath so that an accurate adjustment on the principles explained may be made 65 periodically. Under these conditions the bath may be maintained in a practically uniform state of activity and efficiency. Under the working conditions described the amount of acids added to the bath for purpose of adjustment almost 70 balances the quantity of solution carried out of

the bath mechanically by the paper so that the process described works very economically and simply. After remaining in the acid bath for the required time the box containing the paper is raised above the acid level and allowed to drain for a few minutes under a ventilating hood. It is then transferred to a large bath containing water in which the box is quickly submerged for a few minutes. The box is successively transferred to a series of similar water baths for the purpose of extracting the acid from the paper and eventually placed in running water until completely freed from acid. The first water bath extracts the greater proportion of the acid and when the concentration of acid reaches about 40 per cent. the solution may be run to a storage tank for subsequent recovery of the acids and the series of water baths moved forward to replace the first bath emptied. By adopting the principle of moving the water baths in an opposite direction to the movement of the paper being freed from acid both water and acids are substantially economized. As soon as the paper is completely freed from acid it may be conveniently stored in water indefinitely or it may be immediately used without further treatment as battery separators. If, however, it is intended to make use of the treated paper in a dry state it should be further purified by prolonged boiling in water to free it from any organic sulphates which may have been formed by the concentrated acid treatment.

It has been found that on exposure of the aluminium spacers to the atmosphere after withdrawal from the nitrating bath and in the subsequent water washing process a small amount of oxidation of the aluminium takes place. In order to avoid chemical reaction of this oxide and the nitrating acids it has been found desirable to repolish the aluminium sheets after being dried and before each successive immersion in the nitrating fluid.

The separators described are suitable for use with plates made from sheet lead weighing one pound per square foot or less but for thicker plates carrying a larger amount of active material it may be desirable to provide a larger space between plates for electrolyte and in that case I prefer to use a slightly thicker paper of say 10 mils and corrugate the paper by passing it between corrugated metal rollers heated to about 140 degrees centigrade before the paper is treated with the acids described. The corrugations so made in the paper before aciding become stiff and permanent after acid treatment and provide wider separation between the plates and consequently more space for the electrolyte.

Another variation which I may use is to assemble two or more sheets of paper between each pair of corrugated aluminium sheets before aciding in such a manner that the paper sheets are pressed closely together when they enter the acid bath in order to cement the paper sheets in contact with each other permanently together. The effect of this process is to provide thicker and stronger separators which can be used to support the lead plates very effectively.

I claim:—

1. A method of preparing separate relatively thin sheets of nitrated cellulose which comprises placing in a nitrating bath relatively thin sheets of cellulose fibre paper interleaved with acid-proof spacing sheets provided with projections and recesses giving the nitrating fluid access to both sides of the sheets of cellulose.

2. A method of preparing separate relatively thin sheets of nitrated cellulose which comprises placing in a nitrating bath relatively thin sheets of cellulose in the form of pure cotton fibre paper interleaved with acid-proof spacing sheets provided with projections and recesses giving the nitrating fluid access to both sides of the sheets of paper. 80
- 5 3. A method of preparing separate relatively thin sheets of nitrated cellulose which comprises placing in a nitrating bath relatively thin sheets of cellulose fibre paper which are less than one hundredth of an inch thick interleaved with acid-proof spacing sheets provided with projections and recesses giving the nitrating fluid access to both sides of the sheets of cellulose. 85
- 10 4. A method of preparing separate relatively thin sheets of nitrated cellulose which comprises placing in a nitrating bath relatively thin sheets of cellulose fibre paper interleaved with aluminium spacing sheets provided with projections and recesses giving the nitrating fluid access to both sides of the sheets of cellulose. 90
- 15 5. A method of preparing separate relatively thin sheets of nitrated cellulose which comprises placing in a nitrating bath relatively thin sheets of cellulose fibre paper which when immersed in the bath lie in substantially vertical planes and are interleaved with acid-proof spacing sheets provided with projections and recesses giving the nitrating fluid access to both sides of the sheets of cellulose. 95
- 20 6. A method of preparing separate relatively thin sheets of nitrated cellulose which comprises placing relatively thin sheets of cellulose fibre paper interleaved with acid-proof spacing sheets provided with projections and recesses to give the nitrating fluid access to both sides of the sheets of cellulose, in a holder capable of being lowered into and raised out of a nitrating bath and provided with spaces to allow the nitrating fluid to flow freely into the box among the sheets, immersing said holder in a nitrating bath, and, after nitration transferring the holder with the sheets in it to a washing bath. 100
- 25 7. A method of preparing separate relatively thin sheets of nitrated cellulose which comprises placing relatively thin sheets of cellulose fibre paper interleaved with acid-proof spacing sheets provided with projections and recesses to give the nitrating fluid access to both sides of the sheets of cellulose, in a holder capable of being lowered into and raised out of a nitrating bath and provided with spaces to allow the nitrating fluid to flow freely into the box among the sheets, immersing said holder in a nitrating bath, and, after nitration, transferring the holder with the sheets in it to each of a series of washing baths of successively decreasing acid concentration whereof the first is removed on reaching a certain concentration and replaced by a fresh bath at the opposite end of the series. 105
- 30 8. A method of preparing separate relatively thin sheets of nitrated cellulose which comprises placing relatively thin sheets of cellulose fibre paper interleaved with acid-proof spacing sheets provided with projections and recesses to give the nitrating fluid access to both sides of the sheets of cellulose, in a holder capable of being lowered into and raised out of a nitrating bath and provided with spaces to allow the nitrating fluid to flow freely into the box among the sheets, immersing said holder in a nitrating bath, and, after nitration transferring the holder with the sheets in it to a washing bath. 110
- 35 9. A method of preparing separate relatively thin sheets of nitrated cellulose which comprises placing relatively thin sheets of cellulose fibre paper interleaved with acid-proof spacing sheets provided with projections and recesses to give the nitrating fluid access to both sides of the sheets of cellulose, in a holder capable of being lowered into and raised out of a nitrating bath and provided with spaces to allow the nitrating fluid to flow freely into the box among the sheets, immersing said holder in a nitrating bath, and, after nitration, transferring the holder with the sheets in it to each of a series of washing baths of successively decreasing acid concentration whereof the first is removed on reaching a certain concentration and replaced by a fresh bath at the opposite end of the series. 115
- 40 45 50 55 60 65 70 75 120 125 130 135 140 145 150
- SAMUEL ALEXANDER POLLOCK.